

## UNITED STATES PATENT OFFICE

2,656,309

## PROCESS OF COKING A MIXTURE OF A CARBONACEOUS MATERIAL AND A HIGH BOILING BITUMINOUS PITCH

Walter T. Brown, Pittsburgh, Pa.

No Drawing. Application February 5, 1951,  
Serial No. 209,519

18 Claims. (Cl. 202—33)

1

The present invention relates to a coking process and, more particularly, to a process for producing high quality coke, such as metallurgical coke, from coke fines and polymerized bitumen in a bottom-heated, horizontal retort or coking chamber, without briquetting.

Broadly stated, the present invention relates to a coking process for producing a high quality coke from dried coke fines or braize of less than  $\frac{1}{4}$ " size ( $\frac{1}{4}$ " x 0) or other non-coking bituminous material which is mixed with a high softening point coal tar pitch or other bituminous material composed principally of unsaturated polynuclear hydrocarbons, which mixture is heated in a horizontal retort or coking chamber, the bottom of which is heated sufficiently to cause polymerization of the hydrocarbons and formation of a solid cake of coke. The coal tar pitch (or other bituminous material) when heated becomes liquid and flows, thereby thoroughly wetting all the cells and pores of the coke fines and filling the interstices between the coke particles. Then the high boiling cyclic, polynuclear hydrocarbons are polymerized by heat to form long chain polymers that thoroughly cement the coke particles together. Further heating in the coking retort depolymerizes the mass, with an evolution of some hydrogen and ammonia, whereby the coke particles and the polymerized bitumen coalesce and form a solid cake of high quality coke which physical coke tests show has high shatter and stability properties. This coke may be crushed to any desired size for use in blast furnaces or for other purposes.

The coking process embodying the present invention is limited to the use of a flat, level, horizontal, bottom-heated retort or coking chamber of any design. The coking process cannot be successfully accomplished in a vertical retort or the standard, vertical, slot-type, by-product coke oven (such as Koppers, Wilputte, Semet-Solvay, Otto and others), because the coal tar pitch or other bitumen, when heated, flows toward the bottom of the vertical coking chamber and does not thoroughly wet all the coke particles or fill the interstices between the coke particles, and destructive distillation in a vertical coking chamber causes depolymerization of the coal tar pitch. Hence, a large amount of the coal tar pitch is distilled off, leaving an unconsolidated mass of honeycombed coke particles, which is of no value.

The coking process embodying the present invention is related in no way whatever with any briquetting process, in which a binder of pitch, asphalt, starch, or the like, is used as a binder

or glue, whereby the coke particles, coal fines, anthracite culm, etc., are cemented together by pressure in a briquetting press of any suitable design. The present coking process involves a high softening point coal tar pitch or similar bitumen composed chiefly of polynuclear hydrocarbons, which can be polymerized. This bituminous material would be unsuitable for use as a binder or glue in a briquetting process, because it is brittle and has little cementing properties.

Also, the coking process embodying the present invention should not be confused with processes for producing petroleum coke or pitch coke, in which hot, residual oil or pitch is sprayed into a retort or coking chamber, wherein destructive distillation depolymerizes the residual oil or pitch, leaving a carbon residue, known as petroleum coke or pitch coke, which is used in the manufacture of carbon electrodes.

## 20 Coke fines

Coke fines, also called coke braize or coke breeze, is produced in the manufacture, crushing, handling and quenching of by-product or beehive coke from bituminous coals. In coke plants producing blast furnace coke, the  $\frac{1}{8}$ " x 0 or  $\frac{3}{4}$ " x 0 size is screened out as coke braize or coke fines. There is a considerable quantity of coke fines produced, which is of little or no value.

At some coke plants, the  $\frac{3}{4}$ " x  $\frac{1}{4}$ " size is screened out of the coke braize or fines and sold or used in gas producers or for other purposes. Also, some coke plants burn the coke braize under steam boilers, but the  $\frac{1}{8}$ " x 0 size coke fines are generally not burned and blow out the stacks or settle in the waste gas flues, thereby constitute a waste by-product.

In chemical plants manufacturing calcium carbide in electric furnaces, the by-product or beehive coke is crushed to 1" x 0 size and the 10 mesh x 0 very fine size coke is screened out. There is approximately ten (10%) percent of the 10 mesh x 0 size coke fines which is a waste material. Many attempts have been made at coke and chemical plants to utilize the  $\frac{1}{4}$ " x 0 size coke fines by briquetting and other methods, but these have not been very successful.

Coke has a cellular and porous structure, containing many cells or macro and micro pores or capillaries. The coke fines used in the present invention are  $\frac{1}{4}$ " x 0 size and are of the same porous structure, but contain more macro and micro pores, therefore should be thoroughly dried to remove any moisture from these capillaries or micro pores so the coke can be thoroughly wetted

by the coal tar pitch or other bitumen. Coal tar pitch when heated to 400° F. or higher has a low surface tension. Materials having a low surface tension are better wetting agents. The coal tar pitch or bitumen used in the present invention thoroughly wets and penetrates all the macro and micro pores of the dried coke fines before being polymerized.

#### Coal tar pitch or bitumen

The present coking process is limited to the use of coal tar pitch or other bitumen composed principally of unsaturated polynuclear hydrocarbons of various high softening points. Coal tar pitch is a pyrogenous bitumen, because it is produced from bituminous coals by heat or fire and is composed principally of unsaturated hydrocarbons.

Other pyrogenous bitumen, such as pitches produced from oil-gas tar, water-gas tar, wood or pine tar, lignite tar, shale tar, bone tar, rosin pitch and fatty-acid pitches, are not suitable for use in the present coking process, because none of these pitches contains the high-boiling, cyclic hydrocarbons, which will polymerize and thoroughly cement the coke particles in the coking process.

#### Coal tar and coal tar pitch

Coal tar is produced in by-product coke ovens or retorts of various designs by the carbonization of bituminous coals. The quantity and quality of the coal tar produced depends upon the coals or coal mixture used, design of the coke oven or retort, coking time and carbonization temperature.

Coal tar is a carbon-olesol, that is, a colloidal solution of micro and ultramicro size carbon particles in an oily solution. These carbon particles, when observed under the cardioid ultra-microscope, have a rapid Brownian movement. The finely divided carbon particles are called "micelles" (micelles are the organic molecular aggregates occurring in colloidal solutions) and are the "lyophobic" portion of the colloid solution. The protective bodies are known as the "lyophilic" portion of the system and are composed of heavy hydrocarbon oils, such as anthracene, phenanthrene, pyrene, chrysene and other polynuclear, cyclic hydrocarbons. The light oils, carbolic oils and creosote oils have no value as protective bodies for the micelles and are easily removed by distillation. The micron size is 0.000020 c. m. and the ultramicron size is 0.000001 c. m.

Cardioid ultramicroscope studies of coal tar show that the carbon particles or micelles measure 0.0000148 c. m., which is between the micron and ultramicron sizes. These studies also show that one gram of coal tar contains 513 billion carbon particles or micelles.

Coal tar is commercially distilled in various designs of batch and continuous tar stills and tar heaters in order to recover the light oils, carbolic oils and creosote oils which are the most valuable constituents of coal tar and have a ready market. The residue is coal tar pitch which may be produced to have any desired softening point, depending on the amount of oils distilled off, such as road tars, roofing pitch, briquette pitch, fuel pitch, etc.

When the distillation of coal tar is carried to high-melting point pitches to obtain heavy oils for creosoting or other purposes, a less valuable pitch is obtained, called hard pitch or fuel pitch,

which is best suited for use in the present coking process.

The largest recovery of distillate oils is obtained when coal tar is distilled in a continuous fractionating still under vacuum. When coal tar is distilled in a simple batch still or tar heater, the yield of distillate oils is lower and there is cracking or depolymerization of the residual pitch. The cracking ruptures the protective bodies (heavy hydrocarbon oils), causing the carbon particles to be released and are shown as clusters without Brownian movement in the cardioid ultra-microscope, and laboratory tests shown an increase in "free carbon."

The coal tar pitch used in the coking process embodying the present invention is composed of carbon particles in a medium of high-boiling (above 300° C.) cyclic, polynuclear hydrocarbons.

The cyclic hydrocarbons comprise phenanthrene, anthracene, naphthacene, tetramethyl-anthracene, pyrene, chrysene, picene, etc.

The cyclic hydrocarbons, particularly the tri, tetra and penta cyclic or polynuclear hydrocarbons, are readily polymerized by heat to form giant polymers of high molecular weight. Polymerization is a chemical reaction involving a successive addition of a large number of relatively small molecules (monomers) to form a final compound or polymer.

#### Steps in the coking process

1. In carrying out the present invention, the  $\frac{1}{4}''$  x 0 coke fines (or other non-coking bituminous material) are thoroughly dried by means of a flash dryer, multi-louvre dryer, roto-louvre dryer or other means, to remove the moisture from the cells, or macro and micro pores of the coke fines. This will prevent foaming of the coal tar pitch, or other bituminous material composed substantially of unsaturated, polynuclear, high boiling, cyclic hydrocarbon, and permit the bitumen to flow freely and penetrate into the cells, pores and capillaries of the coke fines and to fill the interstices between the coke particles. The waste flue gases from the coking retort may be used for drying the coke fines, or any other means of heat or hot gases may be used.

2. The coal tar pitch or other bitumen is flaked or crushed to  $\frac{1}{8}''$  x 0 size and blended with the dried coke fines in the proper proportions to produce the quality coke desired.

Successful coking was accomplished with 75%, by weight, of  $\frac{1}{8}''$  x 0 coke fines and 25%, by weight, of coal tar pitch, to produce a high-quality coke with as high as 52 stability factor in the tumbler test.

The coal tar pitch or bitumen may be heated until it is a liquid and sprayed on the hot, dried coke fines, or mixed with the dried coke fines by any desired means. The coating of the coke fines with coal tar pitch will prevent any re-absorption of moisture and produce a mixture of non-coking, bituminous fines and bitumen of the proper proportions for charging into a coking retort. A high-quality coke has been successfully produced by this method.

3. The mixture of dried coke fines and coal tar pitch or other bitumen is charged into a flat, level, horizontal, bottom-heated coking retort or oven chamber of any design, which is heated by gas, oil, tar, pitch or electricity or any other means of heating. Such retorts and ovens, per se, form no part of the invention, being well

known in the art and described in United States patents such as the following:

Hughes, 2,259,380, October 14, 1941;

Hughes, 2,234,173, March 11, 1941;

Knowles et al., 1,885,920, November 1, 1932;

Curran, 2,267,447, December 23, 1941.

The temperature of the bottom of the coking retort should not exceed 1800° F., and best results are obtained between 1400° F. and 1700° F. Higher temperatures distill off the heavy hydrocarbon oils from the pitch before they have a chance to polymerize.

The coking retort must be flat, level, and horizontal, and heated from the bottom only and may be constructed of metal, silica brick, silicon carbide (Carbofrax) or any other suitable heat-resisting material. The ends of the coking retort should have closures or doors, which will hermetically seal the coking retort. A gas off-take should be provided at or near the top of the retort to remove any gas evolved. The gases can be vented to the atmosphere or collected in the conventional by-product recovery apparatus.

4. The heat in the bottom of the coking retort causes the coal tar pitch to melt and flow into all the cells, pores and capillaries of the coke fines and fill in all the interstices between the coke particles. More specifically, the heat from the bottom of the coking retort lowers the surface tension of the coal tar pitch so that it thoroughly wets and penetrates all the cells, pores and capillaries of the dried coke fines.

The heat from the bottom of the coking retort then causes the high-boiling, cyclic, polynuclear hydrocarbons to polymerize within and around the coke particles, thereby producing giant polymers. On further heating the coke fines and the polymerized bitumen coalesce, forming a solid cake of high-quality coke. The unpolymerized or partially polymerized hydrocarbons, etc., are depolymerized with the evolution of hydrogen and ammonia.

5. The coke produced is discharged from the coking retort or chamber by any suitable means.

The depth of the mixture of coke fines and coal tar pitch, or other bitumen, in the flat, horizontal, bottom-heated coking retort is limited by the coking temperature and the amount of coal tar pitch used, but should not exceed 12 inches in depth. However, it is possible that further development of the present coking process may prove that a greater depth of mixture of coke fines and coal tar pitch may be carbonized satisfactorily. Best results have been obtained with depths of 4 to 8 inches.

The coking rate of the present coking process will depend on the coking temperature and depth of charge in the coking retort. High-quality coke has been produced by the present coking process at the rate of 1 inch to 1.5 inches per hour. The present invention, however, is not limited to any specified coking rate.

#### *Other applications of the present coking process*

The coking process embodying the present invention is not limited to the production of metallurgical coke from coke fines and coal tar pitch or other bitumen, because high-quality coke may be produced from mixtures of high, medium or low volatile bituminous coking coals; coke fines; coal tar pitch; or other bitumen.

Also, the present coking process may be utilized for coking a mixture of non-coking or poorly coking coals or chars (such as high volatile "C,"

sub-bituminous, semi-anthracite, anthracite, coal chars or lignite chars) with coal tar pitch or other suitable bitumen.

High quality coke has been produced by the present coking process from the following mixtures (by weight) of bituminous coals, coke fines and coal tar pitch:

1. High volatile coal 25%; coke fines 50%; coal tar pitch 25%.
2. Medium volatile coal 25%; coke fines 50%; coal tar pitch 25%.
3. Low volatile coal 25%; coke fines 50%; coal tar pitch 25%.
4. Medium volatile coal 55%; coke fines 30%; coal tar pitch 15%.
5. Medium volatile coal 60%; coke fines 30%; coal tar pitch 10%.

The above compositions are recited merely by way of illustration and are not to be considered as limiting the scope of the invention inasmuch as variations may be made in the percentages enumerated with satisfactory results.

The present coking process may be utilized in areas away from the bituminous, coking coal producing districts for the production of metallurgical, foundry or domestic cokes from poorly-coking or non-coking coals, or coal fines, or char, which at the present time cannot be utilized for the manufacture of coke.

The use of poorly-coking or non-coking coals, or coal fines, or char for the production of metallurgical or domestic cokes by the present process would conserve the reserves of high quality, coking coals and aid in the economy of the country.

It is desirable to use a mixture of 55% medium-volatile, bituminous coking coal, 30% coke fines and 15% coal tar pitch or other suitable bitumen in the present coking process, in order to supply sufficient coke oven gas for heating the coking retort, to reduce the amount of coal tar pitch (or other bitumen) required and to supply sufficient coal tar for distillation to a high softening point, coal tar pitch. In this way the coking process is self-sustaining and it is not necessary to supply or purchase gas or other fuels for heating the coking retort or coal tar pitch necessary for the process.

However, other mixtures than those specifically recited above may be used in the range of 10% to 60% bituminous coking coals, 10% to 75% coke fines, and 10% to 25% coal tar pitch (or equivalent), by weight.

High-volatile, bituminous, coking coals have a very fluid plastic zone, when being converted from coal to coke, which is readily volatilized during carbonization, leaving a poorly consolidated coke.

Low-volatile, bituminous, coking coals have a very viscous plastic zone when being converted from coal to coke during carbonization, but this plastic zone is very thin and only a small quantity of gas and coal tar is produced during carbonization which would not be sufficient to make the coking process self-sustaining.

Medium-volatile, bituminous, coking coals have a thick, viscous plastic zone when being converted from coal to coke during carbonization. The use of sufficient medium-volatile, bituminous, coking coals in the present coking process with coke fines and coal tar pitch will supply sufficient gas for heating the coking retort, reduce the quantity of coal tar pitch required, and furnish sufficient coal tar for distillation to coal tar pitch to make the coking process self-sustaining and supply light, carbolic and creosote

oils for sale, thereby reducing the operating costs of the coking process.

It should be noted that in the present specification wherever coal tar pitch is specified, other equivalent bitumens, namely, those composed essentially of unsaturated, polynuclear, cyclic hydrocarbons, can be used instead, preferably those having a softening point in excess of 250° F., A. S. T. M. ring and ball (or a melting point of greater than 300° F.) "cube in air method." Also, where coke fines are mentioned, other non-coking, bituminous materials may be substituted therefor.

Thus it will be seen that in accordance with the present invention, there is provided a highly efficient, economical process for making use of coke fines, normally a waste product, which are agglomerated with bituminous material to form a cake of high quality coke, such as metallurgical coke.

While I have illustrated and described several specific embodiments of my invention, it will be understood that these are by way of illustration only, and that various changes and modifications may be made within the contemplation of my invention and within the scope of the following claims.

I claim:

1. A process for producing coke, which comprises mixing dry, non-coking, carbonaceous material with bituminous material composed essentially of unsaturated, polynuclear hydrocarbons having a boiling point in excess of 300° C., and heating the mixture in a horizontal, bottom-heated retort to a temperature to cause polymerization of the hydrocarbons and formation of giant polymers having substantial bonding characteristics.

2. A process for producing coke, which comprises mixing dry coke fines of less than  $\frac{1}{4}$ " particle size with bituminous material composed essentially of unsaturated, polynuclear hydrocarbons having a boiling point in excess of 300° C., and heating the mixture in a horizontal, bottom-heated closed chamber to a temperature below 1800° F. but sufficiently high to cause melting, flow and polymerization of the hydrocarbons.

3. A process for producing coke, which comprises mixing 25% to 75%, by weight, of coke fines of less than  $\frac{1}{4}$ " particle size with 75% to 25%, by weight, respectively, of bituminous material composed essentially of unsaturated, polynuclear, cyclic hydrocarbons having a boiling point in excess of 300° C., and heating the mixture in a bottom-heated, horizontal coke oven at a floor temperature below 1800° F. but sufficiently high to cause polymerization of the hydrocarbons.

4. A process for producing coke, which comprises mixing of the order of 75%, by weight, of coke fines of less than  $\frac{1}{4}$ " particle size with 25%, by weight, of bituminous material composed essentially of unsaturated, polynuclear, cyclic hydrocarbons having a boiling point in excess of 300° C., and heating the mixture in a bottom-heated, horizontal retort at a floor temperature below 1800° F., but sufficiently high to cause polymerization of the hydrocarbons.

5. A process for producing coke, which comprises mixing dry coke fines of less than  $\frac{1}{4}$ " particle size with coal tar pitch having a boiling point in excess of 300° C., and heating the mixture in a bottom-heated, horizontal retort at a floor temperature of the order of 1600° F. to cause polymerization and bonding by the hydrocarbons.

6. The method recited in claim 5 wherein the

coke fines comprise about 75% and the coal tar pitch, about 25%, by weight, of the mixture, and wherein the coal tar pitch is composed essentially of unsaturated, polynuclear, cyclic hydrocarbons.

5. A coking process for producing coke, which comprises mixing thoroughly dried coke fines of less than  $\frac{1}{4}$ " size with ground bituminous material composed essentially of coal tar pitch having a boiling point above 300° C., said coal tar pitch substantially comprising unsaturated, polynuclear, cyclic hydrocarbons, and heating the mixture in a bottom-heated, horizontal retort or coking chamber at a floor temperature of between about 1400° F. and 1800° F. so as to cause polymerization of the hydrocarbons and formation of a solid cake of coke.

20. A process for producing coke, which comprises mixing substantial quantities of bituminous coking coal, coke fines of less than  $\frac{1}{4}$  inch particle size and bituminous material composed essentially of unsaturated polynuclear hydrocarbons having a boiling point in excess of 300° C., and heating the mixture in a bottom heated horizontal coke oven to a floor temperature of the order of 1600° F. to cause polymerization of the hydrocarbons and formation of a solid cake of coke.

25. A process for producing coke, which comprises mixing 10% to 60%, by weight, of bituminous coking coals, 10% to 75%, by weight, of coke fines, and 10% to 25%, by weight, of bituminous material composed essentially of unsaturated polynuclear hydrocarbons having a boiling point in excess of 300° C., and heating the mixture in a bottom-heated, horizontal coking chamber to a temperature below 1800° F. but sufficiently high to cause melting, flow and polymerization of the hydrocarbons.

30. A process for producing metallurgical coke which comprises mixing of the order of 25%, by weight, of bituminous coking coal; 50%, by weight, of coke fines and 25%, by weight, of coal tar pitch comprised essentially of unsaturated polynuclear hydrocarbons having a boiling point in excess of 300° C., and heating the mixture in a bottom-heated, horizontal coking retort at a floor temperature below 1800° F. but sufficiently high to cause polymerization of the hydrocarbons and formation of a cake of coke.

35. A process for producing high quality coke, which comprises mixing about 55%, by weight, of medium-volatile, bituminous coking coal particles, 30%, by weight, of dry coke fines smaller than  $\frac{1}{4}$ " size and 15%, by weight, of particles of coal tar pitch comprised essentially of unsaturated polynuclear hydrocarbons having a boiling point in excess of 300° C., and heating the mixture in a bottom-heated, horizontal coke oven at a floor temperature of between 1400° F. and 1800° F. to cause polymerization of the hydrocarbons and formation of giant polymers having substantial bonding characteristics.

40. A process for producing high quality coke, which comprises mixing about 60%, by weight, of medium-volatile, bituminous coking coal particles; 30%, by weight, of coke fines of less than  $\frac{1}{4}$ " size, and 10%, by weight, of coal tar pitch comprised essentially of unsaturated, polynuclear hydrocarbons having a boiling point in excess of 300° C., and heating the mixture in a bottom-heated, horizontal retort at a floor temperature of between 1400° F. and 1800° F. to cause polymerization of the hydrocarbons and formation of a solid cake of coke.

13. A process for producing coke, which comprises mixing coke fines, bituminous coal and coal tar pitch comprised essentially of unsaturated polynuclear hydrocarbons having a boiling point in excess of 300° C., and heating the mixture in a bottom-heated, horizontal retort sufficiently to melt, flow, wet and penetrate the cells, pores and capillaries of the coke fines and polymerize the unsaturated cyclic polynuclear hydrocarbons of the coal tar pitch and thereby thoroughly cement the coke particles together.

14. A process for producing coke, which comprises mixing 25% to 75%, by weight, of non-coking, bituminous material of less than  $\frac{1}{4}$ " particle size with 75% to 25%, by weight, respectively, of bituminous material composed essentially of unsaturated, polynuclear, cyclic hydrocarbons having a boiling point in excess of 300° C., and heating the mixture in a bottom-heated, horizontal coke oven at a floor temperature below 1800° F. but sufficiently high to cause polymerization of the hydrocarbons.

15. A process for producing coke, which comprises spraying hot, melted bituminous material composed essentially of unsaturated, polynuclear, hydrocarbons having a boiling point in excess of 300° C., upon hot, dried, non-coking bituminous material prior to charging into a horizontal retort, and heating the mixture in a horizontal retort to a temperature to cause polymerization of the hydrocarbons and formation of giant polymers having substantial bonding characteristics.

16. A process for producing coke, which comprises spraying hot, melted coal tar pitch composed essentially of unsaturated, polynuclear, hydrocarbons having a boiling point in excess of 300° C., upon hot, dried, coke fines prior to charging into a horizontal retort, and heating the mixture in a horizontal retort to a temperature to cause polymerization of the hydrocarbons and

10  
formation of giant polymers having substantial bonding characteristics.

17. A process for producing coke, which comprises spraying hot, melted coal tar pitch composed essentially of unsaturated, polynuclear, hydrocarbons having a boiling point in excess of 300° C., upon hot, dried, coke fines prior to charging into a horizontal retort, and heating the mixture in a bottom-heated, horizontal retort or coking chamber at a floor temperature of between 1400° F. and 1800° F. so as to cause polymerization of the hydrocarbons and formation of a solid cake of coke.

18. A process for producing coke, which comprises mixing dry, non-coking, carbonaceous material, and of less than  $\frac{1}{4}$ " particle size, with bituminous material composed essentially of unsaturated, polynuclear hydrocarbons having a boiling point in excess of 300° C., and heating the mixture in a horizontal, bottom-heated, closed chamber to a temperature in the range of about 1400° F. to 1800° F. to cause melting, flow and polymerization of the hydrocarbons.

WALTER T. BROWN.

25

References Cited in the file of this patent

UNITED STATES PATENTS

| Number     | Name          | Date          |
|------------|---------------|---------------|
| Re. 21,651 | Rice -----    | Dec. 3, 1940  |
| 1,308,754  | Graul -----   | July 8, 1919  |
| 1,717,884  | Knowles ----- | June 18, 1929 |
| 1,884,339  | Steere -----  | Oct. 25, 1932 |

35

FOREIGN PATENTS

| Number  | Country             | Date          |
|---------|---------------------|---------------|
| 259,427 | Great Britain ----- | Oct. 14, 1926 |
| 393,297 | Great Britain ----- | May 30, 1933  |
| 884,956 | France -----        | Aug. 13, 1942 |
| 563,366 | Great Britain ----- | Aug. 10, 1944 |

40